

## UNITED STATES PATENT OFFICE

2,249,039

## YARNS AND FABRICS

Herbert Platt, Cumberland, Md., assignor to  
Celanese Corporation of America, a corporation  
of Delaware

No Drawing. Application February 23, 1938  
Serial No. 191,970

12 Claims. (Cl. 28—1)

This invention relates to yarns and fabrics made therefrom and is concerned more particularly with a fabric having a stiffened hand such as an organdy, which hand is acquired solely by the type of yarn employed and is not due to a finish applied thereto. The stiffness of the fabric is substantially permanent, since it is not obtained by the use of finishes which may be removed by either washing or dry cleaning or both.

An object of the invention is the production of fabrics having a stiff hand and especially fabrics of an organdy type. Another object of the invention is the production of an organdy fabric wherein the stiffness is permanent to both washing and dry cleaning. Other objects of the invention will appear from the following detailed description.

Organdy type fabrics are ordinarily produced by weaving yarns or threads of cotton, regenerated cellulose or organic derivatives of cellulose to a ninon or voile. These fabrics are then treated with resins, latex, organic derivatives of cellulose, starch, etc., to effect a stiffness or organdy finish on the fabric. These finishes produce a pleasing effect but they are not permanent to both washing and dry cleaning. Some finishes are not affected by washing but are readily removed by certain organic liquids that may be present in the fluid used by dry cleaners, whereas other finishes are not affected by dry cleaning fluids but are removed or at least partially destroyed by washing in soap and water. Furthermore, any finish applied to a fabric has a tendency to powder-off after long use, especially at places where the fabric is continuously flexed.

I have now found that organdy type fabrics or other stiff fabrics may be made without applying a finish to the fabric. These new fabrics necessarily contain some yarns of organic derivatives of cellulose and the stiffness is due at least in part to the thermoplastic nature of these yarns. Having no finish applied thereto to bind the filaments or fibers of the yarns together the stiffness is permanent, does not powder-off upon flexing of the fabric, and is not affected by either washing and dry cleaning, or both.

In accordance with my invention, I produce a stiffened fabric, especially of the more open weave variety such as organdy, by weaving the fabric from yarns at least some of which are yarns containing an organic derivative of cellulose that have been twisted in the presence of a plasticizing medium to a degree of twist just short of that sufficient to produce a crepe effect upon treating

the fabric in a hot bath. Obviously the degree of twist will vary with the denier of the yarn. However, as a guide to the desired amount of twist, a yarn of 150 denier, 40 filaments may be twisted to between 30 and 50 turns per inch, or referring to the yarn in terms of its twist coefficient (K), obtainable from the formula

$$t = \frac{K}{\sqrt{\text{denier}}}$$

where *t* represents the number of turns of twist per inch, the yarn should have a twist coefficient range of 320 to 600. Also any yarn having a denier between 65 and 250 made of filaments or fibers of a denier below 10 may be twisted from 60 to 20 turns per inch. Such yarn would have a twist coefficient of from 320 to 480, i. e. a yarn having a denier of 250 with a twist of 20 turns per inch would have a twist coefficient of about 320, and yarn having a denier of 65 with a twist of 60 turns per inch would have a twist coefficient of about 480.

Although any plasticizer, gaseous or liquid, may be present during the twisting of the yarns, I have found that good results are obtained if the twisting is effected while the yarn is under the influence of steam, hot water or other heated fluid that has a plasticizing influence on the yarn only at elevated temperatures. For instance, the yarns containing organic derivatives of cellulose may be produced by twisting the yarn on a ring spinning device or upon an upward spinning device by passing the yarn through a steam chamber or through hot water just prior to, during, or just after the insertion of a part of the twist. Preferably a part of the twist should be inserted while the yarn is actually under the influence of the plasticizing medium. The twisting of the yarns may be very conveniently attained by means of the device described in U. S. Patent No. 1,784,581. The twisting operation may also be performed on devices constructed in accordance with the teachings in U. S. Patents Nos. 2,089,778, 2,089,240, 2,089,229 and 2,089,200.

The yarns may be steamed or treated with hot water in the course of one of the twisting operations utilized to apply the requisite twist to the yarn. Conveniently the yarn may be passed through a suitable chamber which may, for instance, take the form of a tube supplied with steam of the desired temperature. If desired, the steam may be applied to the yarn at the point at which the twist is actually applied. For this purpose, where a twisting machine of the type in which twist is applied as the yarn is drawn off

from a bobbin or like package is used, the thread guide immediately above the bobbin from which the yarn is drawn off may be mounted at the point of entry of the yarn into the tube or like chamber in which the steam is applied, or the thread guide may actually be within the said tube or like chamber. Preferably the steam is applied only in the minimum quantity necessary to secure the desired effect on the yarn in order that escape of steam and the consequent likelihood of troubles arising from the rusting of machinery and the like may be avoided as far as possible.

If desired, hygroscopic or deliquescent substances or wetting agents, i. e. agents facilitating the wetting of solids by water, may be applied to or incorporated in the yarns prior to a twisting operation or a steaming or wetting treatment. As examples of such wetting agents may be mentioned soaps of organic or inorganic bases with higher fatty acids, for example, alkali metal, ammonium or ethanolamine soaps, sulphonated oils, sulphonic acids of alkyl naphthalenes for example butyl naphthalene sulphonic acid, and sulphonic acids or sulphuric esters of higher aliphatic alcohols or of mineral oils, tar oils and the like. Mention may also be made of wetting agents of a basic character as, for example, the higher poly-amines of the aliphatic series and basic derivatives of the higher fatty acids, for instance, oleyl derivatives of aliphatic diamines or other higher fatty acid derivatives of this character.

Such hygroscopic or deliquescent substances or wetting agents may be applied to the yarns, or, if desired, may be incorporated in spinning solutions from which the yarns are prepared. For example, cellulose acetate solutions containing hygroscopic substances such as sodium or potassium acetate or calcium or magnesium chloride or nitrate may be spun into filaments and the latter formed into yarns and treated in accordance with the invention. Lubricants, plasticizers and softening agents may also be employed in accordance with the teachings in U. S. Patents Nos. 2,089,241, 2,089,238, 2,089,190 and 2,089,187.

The invention is of particular value in connection with the production of fabrics with the aid of yarns consisting of cellulose acetate filaments. Yarns comprising filaments of other organic derivatives of cellulose may be employed in an analogous manner. As examples of such cellulose derivatives may be mentioned cellulose formate, cellulose propionate or cellulose butyrate or other cellulose esters or organic acids, or methyl, ethyl or benzyl cellulose or other cellulose ethers. If desired, yarns containing both organic derivative of cellulose filaments and filaments of other materials may be employed, for example filaments of silk, cotton, or of artificial silk of the regenerated cellulose type. The yarns may be composed of filaments of two or more different kinds whether in respect of material or denier or both. Thus there may be used threads containing both filaments of cellulose esters or ethers and filaments of natural silk or regenerated cellulose artificial silk, or threads containing cellulose ester or ether filaments of two or more different deniers, or threads containing filaments of one cellulose derivative, e. g. an ester in admixture with filaments of another cellulose derivative, e. g. an ester of different ester content or an ether. Furthermore, the yarns may consist, wholly or in part, of "staple fibre," i. e. relatively short lengths of organic derivative of cellulose filaments.

The yarns may be formed into fabric by any suitable method such as weaving, warp knitting, circular knitting, netting, knotting and the like. The invention is particularly applicable, however, 5 to the formation of fabrics which have a fairly open construction and an organdy stiffness and resiliency, in all respects similar to the organdies made by coating ninon, voile or light weight taffetas with a stiffening material. Such fabrics 10 are formed by weaving in both weft and warp yarns having a denier between 80 and 150. These fabrics may contain from 85 to 135 ends per inch in the warp and from 85 to 105 picks per inch of filling. Fabrics so constructed are of the light 15 organdy type.

The fabric need not be constructed entirely of organic derivative of cellulose yarns twisted as above described. However, the stiffness and resiliency of the resulting fabric will be somewhat proportional to the amount of these yarns employed. It is within the scope of this invention 20 to form fabrics containing organic derivative of cellulose yarns made as described above in conjunction with organic derivative of cellulose yarns containing little or no twist, or twist which has not been set in the presence of a heated fluid or organic derivative of cellulose threads twisted to such a degree that they produce a crepe effect. Furthermore, the organic derivative of cellulose yarns produced as above described may be interwoven with yarns of materials other than organic derivatives of cellulose, such as cotton, silk, wool, linen, etc. The yarns 25 constructed in accordance with this invention may be used in the warp or weft or both when employed in conjunction with other types of yarns. The preferred embodiment, however, is, as stated above, the production of organdy type fabrics composed entirely of organic derivative of cellulose yarns having a set twist produced by twisting the yarns to a high degree of twist in the presence of a plasticizing medium. The twist, however, should not be to such a high degree 30 that it would produce a crepe effect when the fabrics formed therefrom are subjected to a heat bath.

As an illustration of this invention, but without being limited thereto, the following example is given:

#### Example

Cellulose acetate yarns of 100 denier, 25 filaments are twisted 45 turns per inch while being passed through a steam chamber of sufficient distance that the twist as inserted is set therein. These yarns are woven into a fabric having a taffeta weave employing 126 ends per inch in the warp and 88 picks per inch in the filling. The fabric produced is of the organdy type and the stiffness and resiliency is entirely permanent to both washing and dry cleaning. The fabric is free of any appearance of having had a coating applied thereto and may be flexed continuously without losing its stiffness and resiliency.

The term "set twist" as employed hereinafter in the claims is to be construed as meaning a twist which has been set by a setting medium.

It is to be understood that the foregoing detailed description is merely given by way of illustration and that many variations may be made therein without departing from the spirit of my invention.

Having described my invention what I desire to secure by Letters Patent is:

1. A stiffened non-crepe fabric comprising

yarns containing an organic derivative of cellulose, said yarns having a set twist of a twist coefficient of from 320 to 480.

2. A stiffened non-crepe fabric comprising yarns containing cellulose acetate, said yarns having a set twist of a twist coefficient of from 320 to 480.

3. A stiffened non-crepe fabric comprising yarns containing an organic derivative of cellulose, said yarns having a set twist of a twist coefficient of about 320.

4. A stiffened non-crepe fabric comprising yarns containing cellulose acetate, said yarns having a set twist of a twist coefficient of about 320.

5. An organdy type non-crepe fabric having a taffeta weave and composed of yarns containing an organic derivative of cellulose, said yarns having a set twist of a twist coefficient of from 320 to 480.

6. An organdy type non-crepe fabric having a taffeta weave and composed of yarns containing cellulose acetate, said yarns having a set twist of a twist coefficient of from 320 to 480.

7. In a method of producing a non-crepe fabric having stiffness and resiliency, the step of weaving a fabric from yarns containing organic derivatives of cellulose and having a twist of a twist coefficient of from 320 to 480, the twist being set therein by twisting said yarns while under the influence of a hot aqueous medium.

8. In a method of producing a non-crepe fabric having stiffness and resiliency, the step of weaving a fabric from yarns containing cellulose acetate and having a twist of a twist coefficient of from 320 to 480, the twist being set therein by

twisting said yarns while under the influence of a hot aqueous medium.

9. In a method of producing a non-crepe fabric having stiffness and resiliency, the steps of weaving a fabric from yarns containing organic derivatives of cellulose and having a twist of a twist coefficient of from 320 to 480, the twist being set therein by twisting said yarns in the presence of a plasticizer for said organic derivatives of cellulose.

10. In a method of producing a non-crepe fabric having stiffness and resiliency, the steps of weaving a fabric from yarns containing cellulose acetate and having a twist of a twist coefficient of from 320 to 480, the twist being set therein by twisting said yarns in the presence of a plasticizer for the cellulose acetate.

11. In a method of producing a non-crepe fabric having stiffness and resiliency, the step of weaving a fabric from yarns containing organic derivatives of cellulose and having a twist of a twist coefficient of from 320 to 480, the twist being set therein by twisting said yarns while under the influence of a hot aqueous medium and in the presence of a plasticizer for the organic derivatives of cellulose.

12. In a method of producing a non-crepe fabric having stiffness and resiliency, the step of weaving a fabric from yarns containing cellulose acetate and having a twist of a twist coefficient of from 320 to 480, the twist being set therein by twisting said yarns while under the influence of a hot aqueous medium and in the presence of a plasticizer for the cellulose acetate.

HERBERT PLATT.